

## 1

3,554,712

**GASOLINE CONTAINING N-SULFINYL AMINE**  
George C. Lické, Oxford, Mich., assignor to Ethyl Corporation, New York, N.Y., a corporation of Virginia  
No Drawing. Filed Dec. 20, 1968, Ser. No. 785,804  
Int. Cl. C10I 1/22

U.S. Cl. 44—74

10 Claims

### ABSTRACT OF THE DISCLOSURE

Gasoline, containing as an antiknock agent an N-sulfinyl amine compound, is described.

### BACKGROUND OF THE INVENTION

This invention is directed to the use of N-sulfinyl amines as gasoline antiknock agents.

The octane number of a gasoline is improved by addition of an antiknock agent. The most commonly used antiknock agents are organolead compounds such as tetraethyllead. Sulfur containing compounds in gasoline, on the other hand, are generally detrimental to octane number.

The present invention provides a novel, sulfur containing non-metallic organic compound as an antiknock agent.

### SUMMARY OF THE INVENTION

Gasoline containing an antiknock quantity of an N-sulfinyl amine.

### DESCRIPTION OF PREFERRED EMBODIMENTS

An embodiment of this invention is gasoline containing an antiknock quantity of a compound having the formula



wherein  $x$  is an integer from 1 to 4 inclusive, preferably 1 to 2 inclusive, and  $R$  is selected from

- (a)  $C_5-C_{18}$  alkyl groups
- (b)  $C_6-C_{30}$  aryl groups
- (c)  $C_5-C_{18}$  alkenyl groups, and
- (d) alkylene amino groups having the formula



where  $R_1$  and  $R_2$  are independently selected from hydrocarbon alkyl groups having from 2 to about 4 carbon atoms, and  $y$  is 0 to 6. Gasoline which is substantially free of organolead compounds is preferred.

Another preferred gasoline composition contains N-sulfinyl aryl amines having 6 to about 30 carbon atoms. The amount of N-sulfinyl amine compound present in the gasoline ranges from 0.1 to about 10 gram-mols per gallon. The N-sulfinyl mononuclear aryl amines having 6 to 18 carbon atoms are more preferred. N-sulfinyl aniline and N-sulfinyl substituted anilines such as N-sulfinyl toluidine are especially preferred.

The N-sulfinyl amines used in the invention are defined by Formula I above. Methods of preparing these compounds are available in the art. A representative method of preparing these compounds is direct treatment of the parent primary amine with thionyl chloride in a suitable

## 2

solvent. The reaction is illustrated by the following equation:



5 As the equation illustrates, an N-sulfinyl amine is a derivative of a primary amine in which the two amine hydrogens are replaced by the  $=\text{SO}$  radical. In general then, the N-sulfinyl derivative of any suitable primary amine can be used as a gasoline anti-knock in the practice of this invention, provided that it has sufficient solubility in gasoline to effect octane number improvement.

Preferred N-sulfinyl amines are those in which the  $R$  in the Formula I above is selected from the Groups (a)–(d) listed above. N-sulfinyl amines in which  $R$  is a  $C_5-C_{18}$  alkyl group include linear, cyclic, and branched alkyl groups with one or more sulfinyl moieties. Representative examples of N-sulfinyl amines are:

- N-sulfinyl-n-pentylamine,
- N-sulfinyl-n-octadecylamine,
- N-sulfinyl-2-ethyl-n-hexylamine,
- N-sulfinyl-2,4,4,6,6-pentamethyl-n-heptylamine,
- N-sulfinyl cyclohexylamine,
- N-sulfinyl cyclopentylamine,
- N-sulfinyl cyclooctylamine,
- N-sulfinyl laurylamine,
- and the like.

Representative examples of N-sulfinyl alkyl amines having more than one sulfinyl group are:

- 30 N,N'-disulfinyl-1,5-pentanediamine,
- N,N'-disulfinyl-1,10-decanediamine,
- N,N',N'',N'''-tetrasulfinyl-(2,3 methylamine) 1,4 butanediamine,
- 35 N,N',N'''-trisulfinyl-1,6,12-dodecanetriamine
- N,N'-disulfinyl-1,18-octadecanediamine,
- and the like.

N-sulfinyl amines wherein  $R$  in Formula I is a  $C_6-C_{30}$  aryl group can have one or more sulfinyl groups; and  $R$  can be an unsubstituted aryl group, substituted aryl group, alkaryl and aralkyl group, mononuclear as well as polynuclear aryl group. Representative examples of these N-sulfinyl aryl amines are:

- 45 N-sulfinyl-p-cyclohexylaniline,
- N-sulfinyl-2,6-dichloroaniline,
- N-sulfinyl- $\beta$ -naphthylamine,
- N-sulfinyl-4-diphenylamine,
- N-sulfinyl-4-dodecylaniline,
- 50 N-sulfinyl-2,4-didodecylaniline,
- N-sulfinyl-2,4-dimethylamine,
- N-sulfinyl benzylamine,
- N-sulfinyl- $\alpha$ -anthracenylamine,
- N-sulfinyl-2-isopropylaniline,
- 55 N-sulfinyl-4-octadecylaniline,
- N-sulfinyl-2,4,6-triethylaniline,
- N-sulfinyl-N'-phenyl-phenylenediamine,
- N,N'-disulfinyl-4,4'-diphenylamine,
- N,N',N'''-trisulfinyl-1,3,5-benzenetriamine,
- 60 N,N',N'',N'''-tetrasulfinyl-1,2,4,6-benzene tetramine,
- N,N'-disulfinyl-benzidine,
- N,N'-disulfinyl-3,3'-dichlorobenzidine,
- and the like.

More preferred N-sulfinyl aryl amines are those derived from lower aryl mononuclear mono and diamines having from 6 to about 18 carbon atoms. Representative examples of these N-sulfinyl aryl amines are:

N-sulfinyl-2-methylaniline,  
 N-sulfinyl-2-chloroaniline,  
 N-sulfinyl-4-chloroaniline,  
 N-sulfinyl-2-sec-butylaniline,  
 N-sulfinyl-6-tert-butylaniline,  
 N-sulfinyl-2,6-dimethylaniline,  
 N-sulfinyl-2,4-dimethylaniline,  
 N-sulfinylaniline,  
 N-sulfinylphenethylamine,  
 N-sulfinyl-3-dodecylaniline,  
 N-sulfinyl-2,4,6-tribromoaniline,  
 N-sulfinyl-p-anisidine,  
 N-sulfinyl-o-nitroaniline,  
 N-sulfinyl-2,6-di-isopropylaniline,  
 N,N'-disulfinyl-o-phenylenediamine,  
 N,N'-disulfinyl-2-methyl-p-phenylenediamine,  
 N-sulfinyl-2,6-dimethylaniline,  
 N-sulfinyl-3-dimethylaniline,  
 N-sulfinyl-4-dimethylaniline,  
 N-sulfinyl-2,4-di-tert-butylaniline,  
 N,N'-disulfinyl-p-phenylenediamine,  
 and the like.

N-sulfinyl amines where R in Formula I is an alkenyl group include mono- as well as poly-unsaturated alkenyl compounds. Representative examples of these N-sulfinyl alkenyl amines are N-sulfinyl allylamine, N-sulfinyl oleylamine, N-sulfinyl linoleylamine, N-sulfinyl-4-pentenylamine, N-sulfinyl-2-heptenyl amine, N,N'-disulfinyl-6-dodeceny-1,12-diamine, and the like.

N-sulfinyl amines where R is the group represented by



wherein R<sub>1</sub>, R<sub>2</sub> and y are as defined above, are derived from C<sub>2</sub>-C<sub>4</sub> alkylene diamines and polyamines. Representative examples of these types of N-sulfinyl amines are:



and the like.

Mixtures of N-sulfinyl amine compounds described above can also be used in gasoline compositions of the present invention.

Any gasoline suitable for use in internal combustion engines may be used in the practice of this invention. By gasoline is meant a hydrocarbon or blend of hydrocarbons boiling in the range from about 25° C. to about 250° C. which occur naturally in petroleum as well as suitable hydrocarbons manufactured from petroleum, for example, by thermal or catalytic cracking, polymerizing, reforming, and the like. Typical gasolines are listed in Table I.

TABLE I.—HYDROCARBON COMPOSITION OF BASE GASOLINES

| Hydrocarbon type   | Base gasoline |      |      |      |      |       |
|--------------------|---------------|------|------|------|------|-------|
|                    | A             | B    | C    | D    | E    | F     |
| Aromatics, percent | 30.0          | 27.0 | 34.5 | 19.0 | 24.0 | 0     |
| Olefins, percent   | 4.5           | 11.0 | 8.0  | 18.5 | 12.5 | 5     |
| Saturates, percent | 65.5          | 62.0 | 57.5 | 62.5 | 73.5 | 100.0 |

In the handling of gasolines in refineries, tanks, pipelines, etc., the gasoline may pick up traces of organolead compounds. The term "substantially free of organolead compounds" indicates gasoline that has picked up this minor (generally less than about 0.1 gram of lead per gallon) amount of organolead compounds.

The amount of N-sulfinyl amine which is added to the base gasoline to prepare gasoline compositions of the present invention may be varied. The term "antiknock quantity" means an amount of N-sulfinyl amine sufficient to increase the octane number of the base gasoline. Generally from about 0.1 to about 10 gram-mols of the N-sulfinyl amine can be added per gallon of base gasoline. A gram-mol is the molecular weight of the amine expressed in grams. For example, if the N-sulfinyl amine additive has a molecular weight of 100 then gasoline compositions of the present invention could contain as little as 1 gram or as much as 1000 grams of the amine per gallon of gasoline.

The gasoline compositions of the present invention do not require any special method of preparation. The additive can simply be added directly to the gasoline and blended using any conventional blending means. In addition to the novel N-sulfinyl amine antiknock additive, the present gasoline composition may contain other additives provided that they do not adversely affect the function of the N-sulfinyl amine; such gasoline additives include non-organolead antiknock agents such as (cyclopentadienyl)manganese tricarbonyl, antioxidants such as the hindered phenols, dyes, anti-icing additives, carburetor detergents such as fatty acid amino-amides, corrosion inhibitors, metal deactivators, and the like. If desired, antiknock fluids or concentrates may be prepared containing the N-sulfinyl amines and any combination of other additives and/or diluents.

The feature of the present invention is that the N-sulfinyl amines described above are antiknock agents in gasolines. In other words, gasolines containing N-sulfinyl amines have improved octane ratings. This was demonstrated by blending a series of fuels containing from about 0.5% to about 5.0% by volume of certain N-sulfinyl amines. The Research Octane Number (RON) of the base fuel alone and the base fuel containing the sulfinyl additive were determined using the method of ASTM D-908. The antiknock effect was expressed as the difference (ΔRON) between these two Research Octane Numbers. The data obtained for a series of fuel compositions demonstrating this antiknock effect is contained in Table II below.

TABLE II.—N-SULFINYLAMINES IN BASE GASOLINE A

| Example | Additive               | amount of additive (gram-mols/gal.) | RON <sup>1</sup> | ΔRON |
|---------|------------------------|-------------------------------------|------------------|------|
| 1       | None                   | —                                   | 97.65            | —    |
| 2       | N-sulfinylaniline      | 0.5                                 | 98.05            | 0.40 |
| 3       | 1.0                    | 98.20                               | 0.55             |      |
| 4       | 2.2                    | 98.90                               | 1.25             |      |
| 5       | None                   | —                                   | 97.90            | —    |
| 6       | N-sulfinyl-p-toluidine | 0.5                                 | 98.15            | 0.25 |
| 7       | 1.0                    | 98.45                               | 0.55             |      |
| 8       | 5.0                    | 100.40                              | 2.50             |      |
| 9       | N-sulfinylaniline      | 5.0                                 | 100.35           | 2.45 |

<sup>1</sup> Average of two determinations.

The Research Octane Number data of Examples 1-9 simply illustrate the beneficial effect of N-sulfinyl amines in gasoline.

The following examples further illustrate compositions of the present invention. These compositions are prepared by blending the particular N-sulfinyl amine with the particular base gasoline indicated. In each instance the Research Octane Number of the blend containing the N-sulfinyl amine is higher than the Research Octane Number of the base gasoline itself.

TABLE III

| Example | Base<br>gaso-<br>line | Additive                                                                                                                                     | Amount of<br>additive,<br>g./mols./gal. |
|---------|-----------------------|----------------------------------------------------------------------------------------------------------------------------------------------|-----------------------------------------|
| 10      | B                     | N-sulfinyl-n-pentylamine                                                                                                                     | 0.1                                     |
| 11      | B                     | N-sulfinyl-n-octadecylamine                                                                                                                  | 10.0                                    |
| 12      | B                     | N-sulfinyl-2-ethyl-n-hexylamine                                                                                                              | 5.0                                     |
| 13      | C                     | N-sulfinyl-p-tetraacosylaniline                                                                                                              | 4.0                                     |
| 14      | C                     | N-sulfinyl-2,4-diethylaniline                                                                                                                | 2.0                                     |
| 15      | C                     | N-sulfinyl-a-naphthylamine                                                                                                                   | 1.0                                     |
| 16      | D                     | N,N'-disulfinyl-3,3'-dichlorobenzidine                                                                                                       | 1.5                                     |
| 17      | D                     | N,N',N"-trisulfinyl-1,3,5-benzene triamine                                                                                                   | 0.5                                     |
| 18      | D                     | N-sulfinyl-2,6-dimethylaniline                                                                                                               | 0.8                                     |
| 19      | D                     | N-sulfinyl-benzylamine                                                                                                                       | 2.5                                     |
| 20      | E                     | N-sulfinyl-p-tert-butylaniline                                                                                                               | 6.5                                     |
| 21      | E                     | N,N'-disulfinyl-1,3-propane diamine                                                                                                          | 7.2                                     |
| 22      | F                     | $\text{OS}=\text{N}-\text{C}_2\text{H}_4-\overset{\text{H}}{\underset{\text{N}}{\text{C}}}=\text{N}-\text{C}_2\text{H}_4-\text{N}=\text{SO}$ | 8.5                                     |
| 23      | F                     | $\text{OS}=\text{N}-[\text{C}_4\text{H}_8-\overset{\text{H}}{\underset{\text{N}}{\text{N}}}-\text{C}_4\text{H}_8-\text{N}=\text{SO}$         | 9.3                                     |
| 24      | G                     | $\text{OS}=\text{N}-(\text{C}_2\text{H}_4-\overset{\text{H}}{\underset{\text{N}}{\text{N}}})_5-\text{C}_2\text{H}_4-\text{N}=\text{SO}$      | 3.5                                     |
| 25      | G                     | N-sulfinyl-4-pentenylamine                                                                                                                   | 4.1                                     |
| 26      | G                     | N-sulfinyloleylamine                                                                                                                         | 7.6                                     |
| 27      | A                     | N-sulfinyleclohexylamine                                                                                                                     | 8.4                                     |
| 28      | B                     | N-sulfinyllaurylamine                                                                                                                        | 10.0                                    |
| 29      | C                     | N-sulfinyl-4-diphenylamine                                                                                                                   | 0.15                                    |
| 30      | D                     | N,N',N",N'''-tetrasulfinyl-1,6,7,18-octadecyltetramine                                                                                       | 0.3                                     |
| 31      | E                     | N-sulfinyl-N'-phenyl-p-phenylenediamine                                                                                                      | 0.4                                     |

The gasoline compositions of the present invention have been fully described above. Data is presented to show the antiknock effectiveness of the N-sulfinyl amines in these gasoline compositions.

I claim:

1. Gasoline containing an antiknock quantity of a compound having the formula



wherein  $x$  is an integer from 1 to 4 inclusive and  $\text{R}$  is selected from the group consisting of

- (a)  $\text{C}_5\text{-C}_{18}$  alkyl groups
- (b)  $\text{C}_6\text{-C}_{30}$  aryl groups
- (c)  $\text{C}_5\text{-C}_{18}$  alkenyl groups, and
- (d) alkylene amino groups having the formula



wherein  $\text{R}_1$  and  $\text{R}_2$  are independently selected from hydrocarbon alkyl groups having from 2 to about 4 carbon atoms, and  $y$  is 0 to 6.

2. A gasoline of claim 1 wherein said gasoline is substantially free of organolead compounds.

3. A gasoline of claim 2 wherein the quantity of said compound ranges from about 0.1 to about 10 gram/mols per gallon.

4. A gasoline of claim 2 wherein  $\text{R}$  is a  $\text{C}_6\text{-C}_{30}$  aryl group.

5. A gasoline of claim 3 wherein  $x$  is an integer from 1 to 2 inclusive.

30 6. A gasoline of claim 4 wherein  $\text{R}$  is a  $\text{C}_6\text{-C}_{18}$  mono-nuclear aryl group.

7. The gasoline of claim 6 wherein said compound is N-sulfinyl-p-toluidine.

35 8. A gasoline of claim 6 wherein said compound is N-sulfinyl aniline.

9. A gasoline of claim 7 wherein the concentration of said compound is from about 0.5 to about 5% by volume.

10. A gasoline of claim 8 wherein the concentration of said compound is from about 0.5 to about 5% by volume.

40

#### References Cited

##### UNITED STATES PATENTS

2,794,721 6/1957 Bartleson ----- 44-72X  
3,236,887 2/1966 Hooks et al. ----- 260-551S

PATRICK P. GARVIN, Primary Examiner

W. J. SHINE, Assistant Examiner

U.S. CL. X.R.

44-72; 252-386